

## 1

3,623,327

### PROCESS OF GAS GENERATION WITH PROPELLANT ADDITIVE

William A. Duncan, Huntsville, Billy J. Sandlin, Athens, and James A. Murfree, Jr., Huntsville, Ala., assignors to the United States of America as represented by the Secretary of the Army  
No Drawing. Original application July 5, 1967, Ser. No. 651,325. Divided and this application Oct. 28, 1968, Ser. No. 772,069

Int. Cl. C06d 5/10

U.S. Cl. 60—219

2 Claims

#### ABSTRACT OF THE DISCLOSURE

The use of O-methylhydroxylamine as an additive to exothermally decomposing monopropellants to promote the reaction with an oxidizing agent in a gas generation scheme.

#### CROSS-REFERENCE TO RELATED APPLICATION

This application is a division of applicants' copending application Ser. No. 651,325, filed July 5, 1967.

#### BACKGROUND OF THE INVENTION

This invention relates to a propellant additive and in particular to one used in a gas generation scheme employing an exothermally decomposing monopropellant, a suitable oxidizing agent and a porous support material that supports the oxidizing agent, and as more specifically disclosed in application Ser. No. 651,654, filed July 7, 1967 by applicants.

There is considerable interest in the rocket propulsion industry in the development and use of liquid monopropellant gas generators. Although the majority of work in this field has been in catalytic decomposition schemes, recent attention has been focused on "one-shot" schemes of gas generation utilizing a liquid monopropellant and an inert bed or support. In these schemes, the monopropellant reacts with the initiator to start decomposition, generate heat, and heat the support which, when heated, thermally sustains the decomposition.

Accordingly, the principal object of this invention is to improve the "one-shot" gas generation scheme.

Another object of this invention is to improve the burning rates and properties of propellants for use in liquid monopropellant gas generators.

#### SUMMARY OF THE INVENTION

It has been discovered that methoxylamine

(CH<sub>3</sub>ONH<sub>2</sub>)

## 2

more properly known as O-methylhydroxylamine, when used as an additive to hydrazine or other exothermally decomposing monopropellants and when used in liquid gas generators, results in a much more vigorous and faster ignition with an initiator (oxidizing agent).

#### DESCRIPTION OF THE PREFERRED EMBODIMENT

As an example, the reaction of hydrazine containing 50% methoxylamine by weight with both iodic acid and iodic anhydride is more rapid and more vigorous than the corresponding reaction with pure hydrazine.

The synergistic effect of the additive reduces ignition delay upon firing.

Examples of suitable oxidizing agents are iodic acid and iodic anhydride.

The monopropellant must be an exothermally decomposing type so that when decomposed, it liberates heat which raises the temperature of the environment such that the exothermal decomposition of the monopropellant is maintained thermally.

Preferably, the propellant incorporating the O-methylhydroxylamine should contain 25% to 75% O-methylhydroxylamine by weight (in hydrazine).

We claim:

1. A process of producing gases with a liquid gas generator, said process comprising suspending an oxidizer selected from iodic acid and iodic anhydride in an inert bed, and bringing an exothermally decomposing monopropellant consisting of a mixture of hydrazine and O-methylhydroxylamine into contact with said oxidizer suspended in said inert bed to cause said oxidizer and monopropellant to immediately upon contact react vigorously to produce the desired gases and at the same time reduce ignition delay in the liquid gas generator.

2. A process of producing gases as set forth in claim 1, said mixture containing from about 25% to about 75% by weight of O-methylhydroxylamine.

#### References Cited

##### UNITED STATES PATENTS

|    |           |        |                      |          |
|----|-----------|--------|----------------------|----------|
| 45 | 2,925,709 | 2/1960 | Mantell et al. ----- | 60—218 X |
|    | 2,930,184 | 3/1960 | Plescia et al. ----- | 60—218 X |
|    | 3,021,667 | 2/1962 | Griffin et al. ----- | 60—218   |
|    | 3,117,415 | 1/1964 | Greene -----         | 60—215   |

50 BENJAMIN R. PADGETT, Primary Examiner

U.S. Cl. X.R.

60—215; 149—36